

Nov. 19, 1940.

A. B. KINZEL

2,221,949

HANDLING HOT AQUEOUS SOLUTIONS OF PHOSPHORIC ACID

Filed June 13, 1939



INVENTOR  
AUGUSTUS B. KINZEL  
BY  
*E. Greenwald*  
ATTORNEY

## UNITED STATES PATENT OFFICE

2,221,949

HANDLING HOT AQUEOUS SOLUTIONS OF  
PHOSPHORIC ACIDAugustus B. Kinzel, Douglaston, N. Y., assignor to  
Electro Metallurgical Company, a corporation  
of West Virginia

Application June 13, 1939, Serial No. 278,819

6 Claims. (Cl. 23—165)

This invention relates to the art of handling hot aqueous solutions of phosphoric acid and provides a method of handling such solutions in apparatus resistant to corrosion by hot phosphoric acid at temperatures between 200° C. and 400° C.

Phosphoric acid has a diversity of commercial uses. For example, it is used in the manufacture of fertilizers, baking powder, and in the manufacture of phosphates for other purposes.

5 It may also be used as a catalyst in the hydration of olefines. Many difficulties are encountered in the handling of phosphoric acid due to its corrosive properties. Chromium-nickel steels containing about 18% chromium and 8% nickel

10 have been used for handling cold, dilute acid, but are unsatisfactory for use in contact with concentrated acid. In the manufacture of phosphoric acid, lead lined equipment is frequently used, but the use of such equipment is limited

15 because certain concentrations of phosphoric acid attack lead. When the acid is used in the manufacture of food products such as baking powder, the presence of lead in the acid, resulting from its attack on lead equipment, is undesirable since

20 the final product is apt to be contaminated by the lead in the acid. The presence of lead in more than a specified amount in food products is prohibited by Government regulations.

Accordingly, it is desirable that equipment for handling phosphoric acid be fabricated from a material even more resistant to the corrosive action of phosphoric acid than lead. Silver is a material which is resistant to corrosion by phosphates, and steam jacketed silver kettles

25 have been used in the preparation of sodium salts of phosphoric acid. However, Circular C412 of the Bureau of Standards (published October 2, 1936) at page 36 shows that in tests of

30 pure silver in an 85% solution of phosphoric acid at 210° C. to 231° C. over a period of 16 hours, silver was attacked at the rate of 35 to 69 mg./cm.<sup>2</sup>/day. At temperatures of 112° to 121° C. over a period of 28 hours the corrosion rate in 35% phosphoric acid solution was about 3 mg./cm.<sup>2</sup>/day. Thus, while silver is quite resistant to phosphoric acid at temperatures below 200° C. it is rather severely attacked at temperatures above about 200° C.

35 Furthermore, tests which I have conducted have demonstrated that even at moderately elevated temperatures silver readily softens. In addition, at temperatures above about 200° C. the creep strength of silver is negligible. Because 40

45 50 55 of these characteristics silver can safely be used

for the handling of phosphoric acid only at temperatures considerably below 200° C.

It is a principal object of this invention to provide apparatus resistant to phosphoric acid at temperatures above 200° C. It is a further object 5 to provide such apparatus which also retains its strength at elevated temperatures between about 200° C. and 400° C. Another object is a process for handling hot aqueous solutions of phosphoric acid which comprises holding such 10 solutions in a container composed of a silver-silicon alloy resistant to corrosion by phosphoric acid and having high creep strength at elevated temperatures. Another object is to provide apparatus which may be used with safety in the 15 handling of hot phosphoric acid. Other objects will become apparent from the following description and the accompanying drawing, in which the single figure is a representation of a vessel fabricated from an alloy having the desired 20 properties.

The objects of the invention are achieved by the application of my discovery that the addition to silver of a eutectic-forming or precipitation-hardening element such as silicon produces an 25 alloy which retains its strength at elevated temperatures and which also possesses resistance to corrosion by phosphoric acid at such temperatures. This discovery was unexpected and surprising because previous attempts to improve 30 the strength of silver by the addition of the usual hardening agents such as tin and copper resulted chiefly in detrimentally affecting its resistance to corrosion by phosphoric acid.

In accordance with the invention, aqueous solutions of phosphoric acid, at temperatures between about 200° and 400° C., are handled in apparatus such as, for example, a container, which may consist of a tank, a tube or other vessel 35 to be used in handling hot phosphoric acid, is fabricated from a silver base alloy containing silicon in a substantial proportion less than about 5%, the silicon being present in the alloy in such proportion as to impart to the alloy the ability 40 to retain its strength at elevated temperatures and to withstand the corrosive attack of phosphoric acid at such elevated temperatures. The 45 silver content of the alloy should be at least 95% and ordinarily the silicon content should not exceed 2%. Preferably silicon is present in a proportion between 1% and 2%.

In the single figure of the drawing a vessel 50 V is shown for holding phosphoric acid at temperatures elevated between about 200° C. and 55

400° C. The vessel V is fabricated from an alloy containing 1% to 2% silicon, the remainder being substantially all silver.

Another embodiment of the invention is a process for handling phosphoric acid at elevated temperatures between about 200° C. and 400° C. which comprises holding such acid in a container, or passing it through a tube, composed of an alloy of silver and silicon substantially resistant to the corrosive action of phosphoric acid and having high creep strength at elevated temperatures not exceeding about 400° C., the alloy containing a substantial proportion of silicon not in excess of 5% but sufficient to impart high creep strength to the alloy.

The invention thus provides apparatus which may be used with safety in the handling of hot aqueous solutions of phosphoric acid at temperatures not exceeding about 400° C. While a specific embodiment of the invention has been described and shown in the accompanying drawing, the invention is not limited to such specific embodiment but is useful in other forms of apparatus used in handling hot phosphoric acid.

This application is in part a continuation of my co-pending application Serial No. 157,696, filed August 6, 1937.

I claim:

1. In the art of handling aqueous solutions of phosphoric acid at elevated temperatures between 200° C. and 400° C., the improvement which comprises holding such acid in a container composed of an alloy of silver and silicon, said container being substantially resistant to the corrosive action of phosphoric acid, and having high creep strength at such temperatures.

2. In the art of handling aqueous solutions of phosphoric acid at elevated temperatures between about 200° C. and 400° C., the improvement which comprises passing such acid through a tube composed of an alloy of silver and silicon, said tube being substantially resistant to the corrosive action of phosphoric acid, and having high creep strength at such temperatures.

3. In the art of handling aqueous solutions

of phosphoric acid at elevated temperatures between 200° C. and 400° C., the improvement which comprises holding such acid in a container composed of an alloy of silver and silicon, said container being substantially resistant to the corrosive action of phosphoric acid, and having high creep strength at such temperatures, the silicon being present in the alloy in a substantial proportion not exceeding 5%.

4. A process for handling phosphoric acid at elevated temperatures between about 200° C. and 400° C. which comprises holding such acid in a container composed of an alloy of silver and silicon substantially resistant to the corrosive action of phosphoric acid and having high creep strength at such temperatures, silicon being present in the alloy in a substantial proportion not exceeding 5% but sufficient to impart to the alloy high creep strength at elevated temperatures not exceeding 400° C.

5. A process for handling phosphoric acid at elevated temperatures between about 200° C. and 400° C. which comprises passing such acid through a tube composed of an alloy of silver and silicon substantially resistant to the corrosive action of phosphoric acid and having high creep strength at such temperatures, silicon being present in the alloy in a substantial proportion not exceeding 5% but sufficient to impart to the alloy high creep strength at elevated temperatures not exceeding 400° C.

6. A process for handling aqueous solutions of phosphoric acid at elevated temperatures between about 200° C. and 400° C. which comprises holding such solutions in a container composed of an alloy of silver and silicon substantially resistant to the corrosive action of phosphoric acid and having high creep strength at elevated temperatures not exceeding 400° C., said alloy containing 1% to 2% silicon with the remainder substantially all silver, the silicon imparting to the alloy high creep strength at elevated temperatures not exceeding 400° C.

AUGUSTUS B. KINZEL. 45